

# UNITED STATES PATENT OFFICE.

JERRY JAY DUNN, OF ELLWOOD CITY, PENNSYLVANIA, ASSIGNOR TO THE SHELBY STEEL TUBE COMPANY, OF PITTSBURGH, PENNSYLVANIA, A CORPORATION OF NEW JERSEY.

## METHOD OF MAKING STEEL OR ALLOY TUBES.

1,006,186.

Specification of Letters Patent. Patented Oct. 17, 1911.

No Drawing.

Application filed October 8, 1910. Serial No. 586,018.

To all whom it may concern:

Be it known that I, JERRY JAY DUNN, of Ellwood City, in the county of Lawrence and State of Pennsylvania, have invented a new and useful Method of Making Steel or Alloy Tubes, of which the following is a full, clear, and exact description.

My invention relates to the manufacture of steel tubes and more particularly relates to the heat treatment of the material during the operations of forming into cold drawn seamless tubes, shafting, and similar hollow or cylindrical bodies.

The object of this invention is to provide an improved method of treating the steel or alloy during its formation into cold drawn annular bodies such as seamless tubes.

In the making of such seamless tubes the heated billets or metal blanks are pierced at a temperature of from 1200 to 1300 degrees C. The piercing operation is performed with a loss in temperature of less than 100 degrees C., and, unless the wall of the blank for cold drawing is comparatively thin, the later work in the rolling mill is so small as to have little or no effect in breaking down the grain of the metal, so that at the beginning of the cold drawing operations the structure of the steel is coarsely crystalline.

In existing methods used heretofore in making such tubes, the billets, after being pierced, are reduced in cross section and wall thickness and increased in length in a rolling mill, usually immediately after the piercing operation and without reheating the pierced billet. The so-formed tubes after being rolled are pickled, and then subjected to cold drawing operations to further reduce the wall thickness of the tubes and to

form them to the desired diameter, being annealed after each cold drawing operation by heating to a temperature of about 720 degrees C., and then cooling, a temperature which does not affect the structure or alter the grain size of the steel. I have discovered that when such pierced billets or partly formed tubes are annealed at a temperature of from 900 to 950 degrees C., or slightly above the upper critical point, the structure

of the steel is changed and the coarse crystalline structure present before such annealing is modified, being refined into a fine granular structure which structure is not affected nor changed in the later cold drawing and annealing operations, the later an-

nealings being always effected by heating to a temperature ranging from 720 to less than 900 degrees C.

When the material is to receive more than three cold drawing operations to produce the required size it is desirable to repeat the anneal at the refining temperature to break up any micro flaws and prevent their extension in the further cold working.

The advantages of my invention will be apparent to those skilled in the art. By subjecting the metal to the heat treatment as above described, the metal is refined and the coarse crystalline structure of the steel or alloy always present after the piercing operation is altered and changed into a fine granular structure. The desired fine granular structure imparted to the metal by such heat treatment is maintained without substantial change during the subsequent cold drawing operation.

By treating the blanks for cold drawing in accordance with my improved method, longitudinal splitting of the tubes by reason of the cold drawing operations and breakage heretofore caused in subjecting the tubes to the cold straightening operations following the cold drawing steps, are reduced and practically eliminated and tubes of increased strength and superior quality are obtained.

By seamless cold drawn tubes as used in the specification and claims, all hollow cold drawn articles are intended to be covered whether of cylindrical, square or other cross section.

Modifications in the steps of the process may be made within the scope of my invention as defined in the appended claims. The number of such steps may vary, depending upon the thickness of the wall in the pierced blank relative to that of the completed article, and other changes may be made.

I claim:

1. In the manufacture of seamless cold drawn tubes and similar hollow bodies, the steps consisting in annealing the hollow blanks by heating above the upper critical point and then cooling and then subjecting the annealed blanks to a cold drawing operation.

2. In the manufacture of seamless cold drawn tubes and similar hollow bodies, the steps consisting in annealing the hollow

100

105

110

blanks by heating above the upper critical point and then cooling and then subjecting the annealed blanks to the usual cold drawing operations, the drawn tubes being annealed at a temperature not exceeding the upper critical point.

3. In the manufacture of seamless tubes and similar hollow bodies, the steps consisting in annealing hollow billets by cooling after heating above the upper retardation point and then alternately cold drawing and annealing the partly formed tubes in reducing the tubes to the desired wall thickness and diameter, the metal being heated to below the upper retardation point after the cold drawing operations.

4. The method of making seamless tubes and similar hollow bodies consisting in subjecting hollow steel blanks to alternate cold drawing and annealing operations, heating the hollow blanks to above the upper critical point in beginning the annealing operations and heating to temperatures less than the

upper critical point in subsequent annealing operations, repeating the heating operation to above the upper critical point, again cold drawing and annealing, and again annealing heating to below the upper critical point.

5. The method of making seamless tubes and similar hollow bodies consisting in subjecting hollow steel blanks to alternate cold drawing and annealing operations, heating the hollow blanks to 900 degrees C. in beginning the annealing operations and heating to temperatures less than 900 degrees C. in subsequent annealing operations, and repeating the heating operation to above the upper critical point as the final annealing operation.

In witness whereof, I have hereunto set my hand.

JERRY JAY DUNN.

Witnesses:

B. F. GOODRICH,  
M. E. NOLAN.